

## UNITED STATES PATENT OFFICE

WALTER O. SNELLING, OF ALLENTOWN, PENNSYLVANIA, ASSIGNOR TO TROJAN POWDER COMPANY, OF NEW YORK, N. Y., A CORPORATION OF NEW YORK

## PROPELLANT EXPLOSIVE

No Drawing.

Application filed February 19, 1926. Serial No. 89,418.

My invention relates to propellant explosives, of the smokeless powder type, and its object is to produce an improved smokeless and flashless propellant containing nitrostarch. This application is a continuation in part of my application Serial No. 479,097 for "improvements in propellant explosives," filed June 20, 1921.

Efforts have heretofore been made to prepare smokeless powder from nitrostarch by colloidization, the nitrostarch being dissolved in a suitable solvent to form a colloid mass, and this colloid mass being then admixed with suitable inorganic oxidizing agents, such as nitrate of soda, nitrate of ammonia, and the like. I have discovered that valuable smokeless powders may be made from nitrostarch, desensitized sufficiently to be non-detonating, but preserving the size and shape of the original starch granules. I have found further that in employing nitrostarch in the form of individual grains, I may successfully employ in connection therewith a compound which at the moment of burning will reduce the flame temperature, rendering the explosive substantially flashless. I have found also that certain organic or inorganic nitrates, particularly guanidine nitrate, when present in sufficient amounts are satisfactory temperature-reducing agents.

As an illustration of one method of preparing an explosive embodying my invention, I instance the following procedure: To 50 parts of nitrated starch in the form of the separate nitrated grains of a vegetable starch, I add 37 parts of guanidine nitrate in the form of a fine crystal meal or of fine particles obtained by grinding, and thoroughly mix. I then bring about surface colloidization of the nitrostarch granules in the manner set forth in U. S. Letters Patent No. 1,310,969, issued to me, as assignor, July 22, 1919, employing as the colloidizing agent, say, 37 parts of commercial liquid trinitrotoluene. By this procedure, I obtain an intimate mixture of the desensitized nitrostarch granules in their original physical form, admixed with the temperature-reducing agent, which product I

can then press in molds to secure grains of the sizes and shapes used in the preparation of ordinary smokeless powder. These grains may at first be somewhat friable, but after standing for some hours, the grains gain 55 in strength and become quite tough. If desired, this period of aging may be materially shortened by a special hardening treatment, the grains being exposed to a temperature of 60°, or higher, for from thirty minutes to an hour.

I have also employed as a colloidizing agent a mixture of liquid trinitrotoluene and nitroglycerin. In this instance, I proceed as described in the foregoing paragraph and 65 prefer to use the ingredients in the following proportions: 60 parts of nitrostarch, 20 parts of guanidine nitrate, 10 parts of liquid trinitrotoluene, and 10 parts of nitroglycerin.

Instead of desensitizing the nitrostarch granules by surface colloidization, I may employ oil or wax as a desensitizing agent. For example, I may take 15 parts of nitrated starch and mix with this 2 parts of molten 70 paraffin wax, thereafter thoroughly incorporating the desensitized nitrostarch so produced with 83 parts of a suitable temperature-reducing agent, such as guanidine nitrate. As the wax has agglomerating as 75 well as desensitizing properties, the product may be pressed into grains or particles of any desired size or shapes. In this case, as in that previously given, the nitrostarch 80 granules are sufficiently desensitized to be 85 rendered non-detonating, and the result is a highly satisfactory smokeless and flashless propellant explosive.

Instead of paraffin wax as the desensitizing agent, I may desensitize the nitrostarch 90 with a suitable oil, such, for example, as a mineral oil, and add an agglutinant, such as shellac or coumarone resin, in sufficient quantity to bind together the granules of starch and the particles of the nitrate to 95 form a coherent mass and permit molding into "grains." Sufficient oil is used to render the nitrostarch non-detonating. For example, I have obtained satisfactory results 100 by using an amount of oil equal to 10% of

the weight of the nitrostarch used, but I do not wish to be limited to this proportion, as the proportions are capable of variation. So also with agglutinant, various proportions may be used. With coumarone resin, I have successfully employed an amount thereof equal to 20% by weight of the finished product.

In employing nitrostarch desensitized by means of oil, it is not absolutely essential that a special agglutinant be employed. For example, using 12 parts oil-desensitized nitrostarch and 88 parts guanidine nitrate, the latter ingredient being in slightly moist condition, the mixture can be compressed at a high pressure to form dense grains, and serve as an embodiment of my invention.

The proportions of the ingredients may be varied within wide limits, particularly with reference to the relative percentages of nitrostarch and guanidine nitrate. The nitrostarch should preferably constitute from 10% to 50% of the finished powder, but for some purposes it is conceivable that satisfactory results may be obtained outside of this range. I prefer to use from 50% to 90% of guanidine nitrate, but in some instances less could be used. The examples heretofore given indicate preferred percentages of colloiding desensitizing and agglutinating agents, but these also may be varied in amount, the quantities required in any particular case being sufficiently indicated to the explosives chemist by the purposes pointed out above.

For the specific ingredients hereinabove specified, equivalents may be substituted. As the temperature-reducing agent, instead of guanidine nitrate, I may employ other nitrates, organic or inorganic, such, for example, as urea nitrate or ammonium nitrate. The structural formulæ of these nitrates are:

Guanidine nitrate  $\text{NH}_2\text{C}(\text{NH}_2)_2\text{HNO}_3$

Urea nitrate  $\text{O:C}(\text{NH}_2)_2\text{HNO}_3$

Ammonium nitrate  $\text{NH}_3\text{HNO}_3$

Thus, it will be seen that these compounds may be considered to be addition products of ammonia or an amine and nitric acid. For the purposes of the claims, these compounds and their equivalents will be defined as addition products of an amine and nitric acid, within which phrase the addition product of ammonia and nitric acid (ammonium nitrate) is included. Nitroguanidine is also applicable as a temperature-reducing agent. Its formula is  $\text{NH}_2\text{C}(\text{NH})\text{NHNO}_2$ , and therefore both nitroguanidine and guanidine nitrate will be defined in the claims as reaction products of guanidine and nitric acid. Hydrocellulose may also be used in place of the other temperature-reducing compounds with satisfactory results.

As agglutinants, I may use waxy materials, such as those heretofore indicated, or

stearic acid, Japan wax, or other equivalent material. Vegetable, animal or mineral oil or oily materials may be employed as the desensitizing agent. The colloiding agent, where used, may be other organic nitrates or organic nitro bodies than the trinitrotoluene and nitroglycerin mentioned, such for example as dinitrotoluene, nitrobenzene, and mononitronaphthalene. Amylacetate, acetone or the like, may also be used. It will also be understood that I may use any customary stabilizing agent, such as diphenylamine, urea or urethane.

The compacting of my product into grains may be brought about either through the action of pressure alone (as in the manufacture of ordinary black powder) or through the agglutinating effect of superficial colloidization, as described in my Patent No. 1,310,969, heretofore referred to, or through the addition of a specific agglutinant as hereinbefore described. In any case, the nitrostarch granules are rendered non-detonating, are preserved in their original form, and are employed with a suitable oxidizing agent to obtain the smokeless and flashless propellant as described.

I claim:

1. A propellant explosive comprising nitrostarch, desensitized by surface colloidization, and guanidine nitrate.

2. A smokeless and flashless powder comprising desensitized nitrostarch and a temperature-reducing agent, the latter being an addition product of an amine and nitric acid.

3. A smokeless and flashless powder comprising desensitized nitrostarch and an organic temperature-reducing agent, the latter being an addition product of an amine and nitric acid.

4. A smokeless and flashless powder comprising desensitized nitrostarch and a reaction product of guanidine and nitric acid.

5. A smokeless and flashless powder comprising desensitized nitrostarch and guanidine nitrate.

6. The process of rendering nitrostarch smokeless and flashless, which comprises thoroughly mixing nitrostarch with guanidine nitrate in the form of fine particles, and thereafter adding a desensitizing agglutinant and compressing the mixture into "grains" of the desired form.

7. The process of rendering nitrostarch smokeless and flashless, which comprises thoroughly mixing nitrostarch granules with guanidine nitrate, and thereafter bringing about surface colloidization of the nitrostarch granules and compressing the mass into "grains" of the desired form.

8. A smokeless and flashless powder comprising desensitized nitrostarch and a temperature-reducing agent selected from the following group,—guanidine nitrate, am-

70

75

80

85

90

95

100

105

110

115

120

125

monium nitrate, urea nitrate, nitroguanidine.

9. The process of rendering nitrostarch smokeless and flashless, which comprises 5 thoroughly mixing nitrostarch with a material selected from the following group,— guanidine nitrate, ammonium nitrate, urea nitrate, nitroguanidine,—and thereafter adding a desensitizing agglutinant and 10 pressing the mixture into "grains" of the desired form.

10. The process of rendering nitrostarch smokeless and flashless, which comprises thoroughly mixing nitrostarch granules 15 with a material selected from the following group,—guanidine nitrate, ammonium nitrate, urea nitrate, nitroguanidine,—and thereafter bringing about surface colloidization of the nitrostarch granules and 20 pressing the mass into "grains" of the desired form.

WALTER O. SNELLING.

25

30

35

40

45

50

55

60

65